

# UNITED STATES PATENT OFFICE.

GEORGE D. VAN ARSDALE, OF NEW YORK, N. Y.

## METHOD OF PREVENTING DISINTEGRATION OF ANODES.

1,193,741.

Specification of Letters Patent. Patented Aug. 8, 1916.

No drawing.

Application filed August 2, 1915. Serial No. 43,300.

*To all whom it may concern:*

Be it known that I, GEORGE D. VAN ARSDALE, a citizen of the United States, residing at New York, in the county of New York and State of New York, have invented certain new and useful Improvements in Methods of Preventing Disintegration of Anodes, of which the following is a specification.

10 This invention relates to an improved method of use of graphite anodes in the electrolysis of solutions, more particularly copper solutions, as applied in the leaching of copper ores, in such a way that the rapid 15 disintegration, which has heretofore prevented the use of graphite or other insoluble anodes, may be entirely prevented.

Heretofore, to the best of my knowledge, no satisfactory anode, for use in the electrolysis of solutions of copper, particularly of sulphate solutions, has been known. Lead, on the whole, has given the best results for sulfate solutions, while in almost all cases carbon is the only substance that can be employed in chlorid solutions. For sulfate 25 solutions, however, even the best qualities of carbon are eventually destroyed. Graphitized carbons have given satisfactory results with chlorid, but not with sulfate solutions.

30 Practically lead anodes have been used, but these are more or less readily disintegrated and require a high current voltage. Fused and magnetite anodes are also in use, but with these the voltage is high.

35 I have discovered that the disintegration, for example, of graphite or carbon anodes in chlorid, and especially sulfate solutions, is probably almost entirely due to the mechanical disintegrating effect of the bubbles of gas evolved in the pores of the anodes, at their 40 surface, during electrolysis, and that by preventing such evolution of gas, disintegration of the anodes may be entirely prevented. The means which I employ for preventing

45 the evolution of gas, at the anode, is the presence, during electrolysis, of a sufficient amount of a depolarizing agent or agents in the solutions treated. When the depolarizers are present, in sufficient amount, the

oxygen or other gases formed at the anode, 50 which would otherwise be evolved in the free state as bubbles, unite in the nascent state with the depolarizing agents and their evolution in the free state is thereby entirely prevented. As a result, there is no disintegration or other appreciable deterioration of the 55 anodes.

Various depolarizers or combinations of depolarizers may be employed, those preferred being salts of iron in the ferrous condition, or sulfur dioxid, or both together. These may be employed with various anodes, although I prefer to use graphite as my anode material since, when working in this way, the voltage is considerably lower than 60 with other materials. However, by employing depolarizers in sufficient amount with lead anodes, the peroxidation and deterioration of the lead may be prevented.

While the deterioration of anodes hitherto 70 has been most marked with sulfate solutions, there is also deterioration, although to a less degree, with chlorid solutions, and since deterioration may be prevented in both classes of solutions, by my method, I do not wish to 75 confine the application of this invention to any single class of solutions, anodes or depolarizers. It is also probable that where the use of insoluble anodes is needed for solutions of metals other than copper, this 80 reaction will also be valuable in preventing disintegration.

I have found, by experiment, that I can prevent disintegration and deterioration of anodes of either graphite, or lead in both 85 sulfate and chlorid solutions of copper, as well as in solutions in other metals by the use of depolarizers in sufficient amount. I have further found that in all of the above instances, sulfur dioxid or ferrous sulfate 90 forms an efficient depolarizer or that both may be used together with equally good results.

Having thus described the invention, what 95 is claimed as new is:

1. The method of preventing disintegration of anodes in the electrolysis of copper solutions, which consists in electrolyzing

such solutions in the presence at the anode of ferrous sulfate and sulfur dioxid in sufficient amounts to prevent the evolution of free oxygen at the anode.

- 5 2. The method of preventing disintegration of graphite anodes in the electrolysis of copper solutions, which consists in electro-

lyzing such solutions in the presence at the anode of ferrous sulfate and sulfur dioxid in sufficient amounts to prevent the evolution of free oxygen at the anode. 10

In testimony whereof I affix my signature.

GEORGE D. VAN ARSDALE. [L. s.]

Copies of this patent may be obtained for five cents each, by addressing the "Commissioner of Patents, Washington, D. C."